# EUROPEAN PATENT SPECIFICATION

(11) **EP 0 445 953 B1**
(45) Date of publication and mention of the grant of the patent: **23.08.1995**
(21) Application number: 91301574.9
(22) Date of filing: 27.02.1991
(51) Int. Cl.: D21H 17/69, D21H 17/67, D21H 17/68, D21H 17/17, D21H 17/55

(54) **Cationic polymer-modified filler material, process for its preparation and method for its use in papermaking**
Mit kationischem Polymer modifizierter Füllstoff, Verfahren zu seiner Herstellung und seine Verwendung in der Papierherstellung
Matériau de remplissage modifié par un polymère cationique, son procédé de préparation et son utilisation pour la fabrication

(30) Priority: 08.03.1990 US 490909
(43) Date of publication of application: 11.09.1991
(73) Proprietor: MINERALS TECHNOLOGIES INC., New York, New York 10174 (US)
(72) Inventor: Gill, Robert A., Bethlehem, Connecticut 18017 (US)
(74) Representative: Gaunt, Robert John

(56) References cited:
- US-A- 2 865 743

## Description

This invention broadly relates to the field of surface treated inorganic compounds. More particularly, the invention relates to the provision of compositions suitable for use as a papermaking filler material wherein an inorganic base filler material is surface treated with a substance which enhances the performance of the filler in the papermaking process. The invention also relates to a method for improving the papermaking process, especially by reducing the requirement for sizing material and for improving the characteristics of paper produced according to the process.

Adequate internal sizing of alkaline papers is an important issue for most papermakers. Early development of cellulose reactive sizing agents resulted in poor control of sizing with excessive amounts of sizing agent used, resulting in increased wet-end deposits, press picking, and in coefficient of friction problems with the paper surface. Problems still occur, mainly due to the overuse of sizing materials. The problems are caused by high surface area materials (e.g., filler and fines) found in the wet-end, which adsorb the size and render it ineffective.

The purpose of internal sizing is to impart resistance to liquid penetration to the sheet. Internal sizing, along with sheet porosity (which is controlled at the size press), controls ink penetration in printing and writing papers, along with binder migration in coating basestock. The sizing of alkaline papers with cellulose reactive sizing agents or "synthetic sizes" has been established for more than 30 years. Two synthetic sizes presently in commercial use, alkyl ketene dimer (AKD) and alkenyl succinic anhydride (ASA), impart sizing to the sheet by means of a chemical reaction (covalent bonding) with the hydroxyl groups of cellulose fiber.

All commonly used untreated fillers (e.g., clay, titanium dioxide, calcium carbonate) are known to have a detrimental effect on sizing. Studies of alkaline papers filled with various types of calcium carbonate have revealed strong inverse correlations between filler specific surface area and internal sizing values in the sheet measured by the Hercules size test (HST). In circumstances where increasing the filler content would be advantageous, associated sizing problems have occurred affecting sheet quality, machine performance, and runnability.

US 2,865,743 discloses a sizing composition comprising silica particles with a ketene dimer deposited on the surface. The composition is prepared by dispersing a ketene dimer or mixture of ketene dimers on a carrier comprising finely-divided amorphous silica to form a free-flowing powder in which the particles of silica contain a deposit or coating of the ketene dimer.

Specially modified precipitated calcium carbonate (PCC) fillers, which can be synthesized at an on-site PCC plant, have been developed to make the sizing of filled sheets more economical and efficient. Laboratory results have shown that by using a chemically modified PCC filler, which has been surface treated with a cationic polymer, the amount of sizing agent can be reduced by one-half while improving other properties as well.

It has been discovered that the addition of certain cationic resin materials to papermaking filler materials such as calcium carbonate, either ground natural calcium carbonate from limestone, or precipitated, greatly enhances the performance of the filler material and results in a paper requiring the addition of substantially less wet end sizing agent, and having excellent opacity and tensile strength properties.

Fig. 1 is a plot of Hercules size measurement versus filler content for handsheets containing modified and unmodified fillers.

Fig. 2 is a plot of water pick-up as measured by the Cobb size test versus filler content for handsheets containing modified and unmodified fillers.

Fig. 3 is a plot of Hercules size measurement versus filler content for handsheets containing modified filler at various levels of polymer treatment.

Fig. 4 is a plot of Hercules size measurement versus filler content for handsheets containing modified and unmodified fillers at different sizing levels.

Fig. 5 is a plot of sheet opacity versus filler content for handsheets containing modified and unmodified fillers.

Fig. 6 is a plot of sheet opacity versus sheet tensile strength for handsheets containing modified and unmodified fillers.

Fig. 7 is a plot of sheet brightness versus filler content for handsheets containing modified and unmodified fillers.

Fig. 8 is a plot of Hercules size measurement versus filler content for sheets containing modified and unmodified fillers made on a pilot papermachine.

Fig. 9 is a plot of water pick-up as measured by the Cobb size test versus filler content for sheets containing modified and unmodified fillers made on a pilot papermachine.

Fig. 10 is a plot of corrected sheet opacity versus filler content for sheets containing modified and ummodified fillers made on a pilot papermachine.

Fig. 11 shows comparative microscopic photographs illustrating distribution of filler material for sheets containing modified and unmodified fillers made on a pilot papermachine.

Fig. 12 represents a three-dimensional plot of Hercules size measurement versus treatment temperature and percent cationic polymer treatment level at an 8% filler level in the handsheets.

Fig. 13 represents a three-dimensional plot of Hercules size measurement versus treatment temperature and percent cationic polymer treatment level at an 16% filler level in the handsheets.

Fig. 14 represents a three-dimensional plot of Hercules size measurement versus treatment temperature and percent cationic polymer treatment level at an 24% filler level in the handsheets.

The cationic polymers found to be most effective for surface treating the papermaking filler materials are dimers of the general formula:
where R is a hydrocarbon group selected from the group consisting of alkyl with at least 8 carbon atoms, cycloalkyl with at least 6 carbon atoms, aryl, aralkyl and alkaryl. Specific dimers are octyl-, decyl-, dodecyl-, tetradecyl-, hexadecyl-, octadecyl-, eikosyl-, dokosyl-, tetrakosyl-, phenyl-, benzyl-beta-naphthyl-, and cyclohexyl- dimer. Other utilizable dimers are dimers produced from mining acids, naphthenic acid, delta-9,10-decylenic acid, delta-9,10 dodecylenic acid, palmitoline acid, olein acid, ricine olein acid, linoleate, linoleic acid, and olestearic acid, as well as dimers manufactured from natural fatty acid mixtures, such as are obtained from cocoanut oil, babassu oil, palm seed oil, palm oil, olive oil, peanut oil, rape seed oil, beef suet and lard, and mixtures of the above.

The polymer is made cationic as a result of treating the dimer with a polyamino-amide and/or polyamine polymer reacted with an epoxidized halohydrin compound, such as epichlorohydrin, thereby forming tertiary and quaternary amine groups on the dimer surface. It is preferred that the cationic charge on the dimer be derived primarily from quaternary amine groups. A polymer material of this type is manufactured by and is commercially available from Hercules, Inc., Wilmington, DE, under the tradename Hercon.

It has been discovered that the use of from about 0.1% to about 10.0% by weight of the cationic polymer material on a filler significantly enhances filler performance in terms of a reduction in the requirement for the addition of wet end sizing agent and an improvement in the optical and physical properties, particularly opacity, Z-directional filler distribution and tensile strength, of the resulting paper in which the filler is utilized.

For the case of utilizing clay as a filler material, it has been discovered that surface treatment of the filler with from about 1.0 to about 2.0 weight percent of a cationic polymer material of the aforesaid type is effective in producing a filler clay having a substantially reduced sizing demand.

It has also been discovered that surface treatment of a PCC filler material with from about 0.25 to about 2.0 weight percent of a cationic polymer material of the aforesaid type is effective in producing a filler having a substantially reduced sizing demand.

Other filler materials, such as titanium dioxide, talc and silica/silicate pigments, which if used untreated have a detrimental effect on sizing, are utilizable when treated with a cationic polymer material of the aforesaid type according to the present invention.

For all types of fillers, it has been discovered that the amount of cationic polymer required to be added to the filler material-containing slurry is directly correlated with the surface area of the filler material.

It has further been discovered that the temperature at which the filler material is treated with the cationic polymer is also a significant parameter in determining the extent to which the sizing demand of the polymer-treated filler is reduced.

Generally, treatment of the aqueous slurry containing the filler material with the cationic polymer is done at a temperature of from about 5 to 70°C. The preferred treatment temperature range is from about 20 to 30°C, and the most preferred treatment temperature is at about 25°C.

It has still further been discovered that the pH of the aqueous slurry containing the filler material has an effect on treatment. The slurry should not be at a pH greater than 10 at the time of the treatment. The filler material treated with the cationic polymer should also subsequently be stored at a pH not greater than 10 to prevent decomposition of the cationic polymer coating which occurs at pH's greater than about 10.

The nature and scope of the present invention may be more fully understood in view of the following non-limiting examples, which demonstrate the effectiveness of cationic polymer modified filler materials.

### Example 1

### Preparation and Comparative Testing of Handsheets Containing Modified and Unmodified Fillers

Comparative Formax (Noble and Wood) handsheets (60 g/m² or 40 lbs./3300 ft²) were prepared from a furnish consisting of 75% bleached hardwood and 25% bleached softwood Kraft pulps beaten to 400 Canadian Standard Freeness (CSF) at pH 7.0 in distilled water. A high molecular weight, medium charge density, cationic polyacrylamide (PAM) retention aid was used at 0.05%. Synthetic sizing agents (AKD or ASA) were added at levels from 0.10% to 0.30%. Several fillers were used, including various polymer-modified PCC fillers to test the effect of the polymer treatment against unmodified PCC and fine ground limestone (FGL). The fillers were added to the furnish at 20% solids to achieve 8%, 16%, 24% and 40% filler in the finished sheets. In addition, a blank, containing no filler was prepared and tested. Distilled water was used throughout the handsheet process. The sheets were conditioned at 50% RH and 23°C and tested for grammage, percent filler, HST, Cobb size, opacity, brightness, caliper, tensile, and porosity. Scattering coefficients were determined using the appropriate reflectance values and Kubelka-Munk equations. Elemental mapping of the filler distribution in the sheet, both in the XY plane and in the Z-directional plane, was performed using a scanning electron microscope (SEM) with elemental analysis capabilities.

Sizing values (HST and Cobb) for sheets filled with the modified PCC fillers were significantly improved, with higher levels of polymer on the PCC providing significantly better sizing at all loading levels greater than 10% versus a low sizing demand filler (e.g., FGL) (Figs. 1, 2, and 3). Comparable sheets can be made using one-third less sizing agent when a 0.5 percent by weight cationic polymer-treated PCC filler was used (Fig.4), and as the graph reveals, even less sizing agent was needed using a 1.0 percent by weight cationic polymer-treated PCC filler. Table I also shows the efficiency of polymer treatment of the filler.

A secondary benefit derived from the modified fillers was an increase of one-half point in opacity without a subsequent loss in tensile strength or sheet brightness (Figs. 5, 6, and 7). The increased opacity without loss of strength or brightness appears to be predominately due to the substantial increase in the cationic charge of the modified filler particles. Increasing the cationic charge on the particles makes them adsorb more uniformly on the fiber surface and less between fiber crossings. Scanning electron micrographs revealed better distribution of the filler in the sheet for the modified PCC fillers which supports improved optical performance. Table II shows the relationship between the filler's specific surface area and polymer treatment level on sizing values.

At higher surface area, more polymer is needed to cover the surface and provide improved sizing. Unexpectedly, as the filler level is increased in the sheet, the sizing values continue to rise for all but the highest surface area filler. This indicates that by the method of treatment of this invention, increased sizing is maintainable through the use of higher filler levels in the sheet. This condition cannot be achieved by the use of untreated fillers.

### Example 2

### Evaluation of Modified PCC Fillers for Retention and Drainage.

A vacuum drainage jar apparatus was used to measure the retention and drainage characteristics of the fillers under conditions similar to an actual high-speed paper-machine. The furnish was the same as used in Example 1 with the retention aid level evaluated at 0.05%. The fillers were added so that a content of 16% +/- 1.0% would be retained in the final pad. The stock (0.5% consistency) was agitated in a three vane jar at 750 rpm. Automatic control placed the contents of the jar under a vacuum of 10 kPa during initial drainage followed by 5 seconds of high vacuum (50 kPa). The pad which formed was weighed and then dried and reweighed to yield percent sheet dryness values (these numbers predict the ease at which water is removed from the sheet). Percent filler retention was calculated from the amount of calcium carbonate in the fiber pad via X-ray fluorescence and the known amount added to the stock.

Improved papermachine runnability can be measured in many ways. Improved drainage on the wire along with increased sheet dryness off the couch provides the paper-maker with the opportunity to increase machine speed (increase production rate) and/or decrease steam consumption at the dryers (increased profitability). Improved filler retention without the need to use excessive amounts of retention aid enhances sheet quality which includes formation. This also leads to better runnability and economics from a cleaner wet end system. Retention and drainage results, shown in Table III, using a vacuum drainage jar revealed improved first pass filler retention for the modified PCC fillers.

Sheet dryness values were also improved over the untreated PCC filler, indicating better drainage. The experiments were conducted under precise and well-controlled conditions in the laboratory, however these results are transferable to a papermachine leading to better wet end control with improved runnability, as is shown in Examples 3 and 4, following.

### Example 3

### Comparative Testing of Furnishes Incorporating Both Modified and Unmodified Fillers on Actual Pilot Papermachine.

A pilot machine run was conducted utilizing a pilot scale papermachine. A 60 g/m² (40 lbs./3300 ft²) sheet was produced using the same furnish composition as in Examples 1 and 2. The same cationic retention aid was utilized at 0.0125% and an AKD sizing agent was added at 0.15%. Various calcium carbonate fillers (i.e., untreated commercial PCC, untreated commercial FGL, 0.5 and 1.0 percent by weight cationic polymer-modified PCC's) were added to achieve levels of 8%, 16%, and 24% filler in the sheet.

The paper was tested for the same properties as in Example 1.

The fillers were characterized with respect to particle size by gravity sedimentation analysis using a Micromeritics Sedigraph 5000D. Specific surface area was determined by the use of BET nitrogen adsorption analysis. Dry brightness was measured using a Hunter LabScan. Particle charge (zeta potential) was determined using doppler laser light scattering technique from a Coulter DELSA 440. Filler properties are listed in Table IV.

Results from the pilot papermachine corroborated the results from the handsheet work. Sizing values shown in Figs. 8 and 9 reveal the improved sizing performance for the modified PCC fillers. Since the Hercules size test (HST) was not sensitive enough to distinguish between sizing differences at the low end, the Cobb test was used to better ascertain their performance. The Cobb sizing test results show the characteristic increase in water pick-up for the commercial fillers (i.e., FGL and PCC) with increasing filler loading. This increase is virtually eliminated when utilizing the modified PCC fillers. In addition, 1.0 percent by weight cationic polymer-modified PCC filler provides essentially the same resistance to water pick-up at all filler loading levels as the unfilled sheet using the equivalent amount of sizing agent. Print quality evaluated through microscopic analysis of half-tone dots shows a marked improvement in ink hold-out in sheets using the modified PCC fillers.

There was a one-half point improvement in opacity, corroborating laboratory results (Fig. 10). Calcium elemental mapping of the filler distribution in the sheet (Fig. 11) revealed better distribution, especially in the Z-directional plane, for the modified PCC fillers.

### Example 4

### Comparative Testing of Furnishes Incorporating Both Modified and Unmodified Fillers on a Production Papermachine.

A mill trial was conducted utilizing a Fourdrinier papermachine running at 610 m/min (2000 fpm). A 60 g/m (40 lbs/3300 ft) high opacity sheet was run with and without a modified PCC filler as part of the furnish composition. The modified PCC filler was treated with 1.5 percent by weight of cationic polymer. An anionic retention aid was utilized along with an ASA sizing agent. Both additives were held constant throughout the trial. Handbox and white-water tray samples were obtained throughout the trial and analyzed for first pass filler retention and total retention. These results are shown in Table V.

Significant improvement in both filler retention and total retention were realized. Z-directional distribution of the modified filler through the sheet was also greatly improved. Better distribution of the filler means less two-sidedness, better dimensional stability and better printability of the paper with less associated whitening and dusting (Table V). Paper samples were tested and revealed a 263% improvement in sizing (i.e. 40 sec. vs. 11 sec.) and equivalent opacity with 4.5% less PCC (i.e. 15.0% vs. 15.7%) and 25% less TiO₂ (0.6% vs 0.8%). A 9% improvement in tensile strength was also realized. These results are shown in Table VI.

**TABLE VI**

| **Physical Properties from Mill Trial** | | |
|---|---|---|
| | Untreated Commercial PCC | 1.5 Wt.% Cationic Polymer-Modified PCC |
| Basis Weight g/m² (lb/3300 ft) | 58.5 (39.0) | 60.15 (40.1) |
| PCC (%) | 15.7 | 15.0 |
| TiO₂ (%) | 0.8 | 0.6 |
| Total Filler (%) | 16.5 | 15.6 |
| Corrected Opacity (%) | 88.3 | 88.2 |
| Machine Direction Breaking Length (km) | 7.77 | 8.50 |
| Hercules Size Test (sec.) | 11 | 40 |

Loss of sizing, referred to as "fugitive sizing", was evaluated after 5 weeks (35 days). The results are shown in Table VII.

**TABLE VII**

| **Fugitive Sizing Results from Mill Trial (Reel No. 6 and 10)** | | |
|---|---|---|
| | Untreated Commercial PCC | 1.5 Wt.% Cationic Polymer-Modified PCC |
| Hercules Size Test (sec) (initial testing) | 9 | 37 |
| Hercules Size Test (sec) (35 days later) | 7 | 36 |
| Percent Change in Sizing (%) | -22 | -3 |

The samples showed a minimum loss of sizing compared to typical commercially filled sheets. The surface coefficient of friction of the sheets was also evaluated. The surface coefficient of friction of the sheets is an important measure of the runnability of the paper through high-speed reprographic equipment. The results of this evaluation are shown in Table VIII.

The polymer-modified PCC-filled sheets showed a better coefficient of friction of the sheet surface than the unmodified sheets.

### Example 5

### Effect of Filler Treatment Temperature on Sizing Demand Reduction at Various Levels of Cationic Polymer Treatment and Filler Loading

A handsheet study was performed to evaluate the effect of filler treatment temperature, that is, the temperature at which the cationic polymer is applied to the filler material, on reduction in the sizing demand in the handsheets utilizing the cationic polymer-treated filler. Treatment was at temperatures in the range of from 25-65°C. Treatment was performed at levels of from 0 to 1.25 weight percent of cationic polymer. The cationic polymer used was an alkyl ketene dimer, Hercon-85 (Hercules, Inc., Wilmington, DE). The filler was a precipitated calcium carbonate (PCC) (Albacar HO, Pfizer, Inc., New York). Filler loading in the handsheets was at several levels, of from 8 to 24 weight percent of treated filler.

Twenty separate surface treatments were performed using four treatment levels (0.5, 0.75, 1.0 and 1.25 wt %) and five treatment temperatures (25, 35, 45, 55 and 65°C), along with an untreated control sample, as shown in Table IX.

All treatments were performed using 10 minutes of low-shear mixing time per sample. Elevated temperatures were maintained for approximately 4 hours before samples were allowed to cool.

Comparative Formax (Noble and Wood) handsheets (60 g/m² or 40 lbs./3300 ft²) were prepared from a furnish blend consisting of 75% bleached hardwood and 25% bleached softwood Kraft pulps beaten to a consistency of 0.3125% and a Canadian Standard Freeness (CSF) of 400 ±25 at pH 7.0 in distilled water. Additional wet end additives included an alkyl ketene dimer size (Hercon-75, Hercules, Inc., Wilmington, DE) in an amount of 0.25 wt. % (2.2 kg/tonne or 5 lb/ton of paper) and a cationic polycacrylamide retention aid (Percol-175) in an amount of 0.05 at % (0.45 kg/tonne or 1 lb/ton of paper). All sheets were conditioned and tested at standard TAPPI conditions of 50% relative humidity and 23°C.

Paper properties tested include size, opacity, pigment scattering coefficient and sheet brightness. Size was tested by the Hercules Size Test. Reported values are in seconds. Opacity was tested by the TAPPI test. Reported values are Corrected opacity, %. Sheet brightness was tested by the TAPPI test. Reported values are Brightness, %. The results are reported in Table X.

The results show that HST values are directly proportional to filler treatment level, that is, the higher the treatment level, the higher the HST response, and inversely proportional to treatment temperature, that is, the higher the slurry treatment temperature, the lower the HST response. Thus, the highest sizing values (greatest sizing demand reduction) occurred at high treatment level and low treatment temperature, while low treatment level and high treatment temperature resulted in poorer size reduction performance. The magnitude of the effect varied considerably, however, with filler level in the handsheets. This is shown in Figures 12, 13 and 14. In Fig. 12, at an 8% filler level, the effect of both treatment level and treatment temperature on HST is minimal, with HST values ranging from a low of 193 seconds to a high of 237 seconds. In Fig. 13, at a 16% filler level, the effect is more noticeable, with HST values ranging from 35 seconds to 392 seconds. Finally, as is seen in Fig. 14, at a 24% filler level, a significant effect is seen, with HST values ranging from 2 to 313 seconds and a very steep transition occurring from lower to higher treatment levels and higher to lower treatment temperature. Treatment level is, however, a more sensitive variable than treatment temperature since a small change in treatment level produces a more drastic HST shift than does a small change in temperature.

## Claims

1. A composition which comprises a papermaking filler material selected from the group consisting of finely ground natural calcium carbonate from limestone, precipitated calcium carbonate, clay, titanium dioxide, talc, silica/silicate pigments, and combinations of the above, which filler material has been surface treated with from about 0.1 to about 10.0 weight percent of a cationic polymer, based on the dry weight of filler material, wherein the cationic polymer is a dimer of the general formula where R is a hydrocarbon group selected from the group consisting of alkyl with at least 8 carbon atoms, cycloalkyl with at least 6 carbon atoms, aryl, aralkyl and alkaryl, the dimer having been made cationic by treatment with at least one of a polyamino-amide and a polyamine polymer reacted with an epoxidized halohydrin compound to form tertiary and quaternary amine groups on the dimer surface.

2. The composition according to claim 1, wherein the dimer is selected from the group consisting of octyl-, decyl-, dodecyl-, tetradecyl-, hexadecyl-, octadecyl-, eikosyl-, dokosyl-, tetrakosyl-, phenyl-, benzyl-beta-naphthyl-, and cyclohexyl- dimers, dimers produced from mining acids, naphthenic acid, delta-9,10-decylenic acid, delta-9,10-dodecylenic acid, palmitoline acid, olein acid, ricine olein acid, linoleate, linoleic acid, and olestearic acid, and dimers manufactured from natural fatty acid mixtures, such as are obtained from cocoanut oil, babassu oil, palm seed oil, palm oil, olive oil, peanut oil, rape seed oil, beef suet and lard, and mixtures of the above.

3. The composition according to claim 1, wherein the epoxidized halohydrin is epichlorohydrin.

4. A process for the preparation of a papermaking filler material surface treated with a cationic polymer, which process comprises adding from about 0.1 to about 10.0 weight percent of a cationic polymer, which is a dimer of the general formula where R is a hydrocarbon group selected from the group consisting of alkyl with a least 8 carbons atoms, cycloalkyl with at least 6 carbon atoms, aryl, aralkyl and alkaryl, which has been made cationic by treatment with at least one of a polyamino-amide and a polyamine polymer reacted with an epoxidized halohydrin compound to form tertiary and quaternary amine groups on the dimer surface, to a filler slurry containing from about 1% to about 76% solids, while maintaining the slurry under agitation at a temperature of from about 5°C to about 70°C, and at a pH less than about 10, in order to improve filler performance.

5. The process according to claim 4 wherein the amount of polymer added to the slurry is directly correlated with the surface area of the filler material.

6. A method for improving papermaking by accomplishing at least one of the results of reducing the amount of sizing required, maintaining the sizing content over time, improving the handling properties of a formed paper web, including water release, improving the physical properties of the resulting paper, including filler retention, filler distribution, tensile strength, and surface coefficient of friction, and improving the optical properties of the resulting paper, including brightness, opacity, and pigment scattering coefficient, which method comprises adding from about 5 to about 50 weight percent of a filler material which has been surface-treated with from about 0.1 to about 10.0 weight percent, based on the dry weight of filler material, of a cationic polymer, which is a dimer of the general formula where R is a hydrocarbon group selected from the group consisting of alkyl with at least 8 carbon atoms, cycloalkyl with at least 6 carbon atoms, aryl, aralkyl and alkaryl, which has been made cationic by treatment with at least one of a polyamino-amide and a polyamine polymer reacted with an epoxidized halohydrin compound to form tertiary and quaternary amine groups on the dimer surface to a papermaking furnish.

## Patentansprüche

1. Zusammensetzung, umfassend einen Füllstoff zur Papierherstellung, ausgewählt aus der Gruppe, bestehend aus feingemahlenem, natürlichem Calciumcarbonat aus Kalkstein, gefälltem Calciumcarbonat-, Ton-, Titandioxid-, Talc-, Silica/Silicat-Pigmenten sowie Kombinationen davon, welcher Füllstoff oberflächenbehandelt wurde mit etwa 0,1 bis etwa 10,0 Gewichtsprozent eines kationischen Polymers, bezogen auf die Trockenmasse des Füllstoffes, wobei das kationische Polymer ein Dimer der allgemeinen Formel ist: worin R eine Kohlenwasserstoffgrupppe ist, ausgewählt aus der Gruppe, bestehend aus Alkyl mit mindestens 8 Kohlenstoffatomen, Cycloalkyl mit mindestens 6 Kohlenstoffatomen, Aryl, Aralkyl und Alkaryl, und das Dimer kationisch gemacht wurde durch Behandlung mit mindestens einem Polyamin-Amid und einem Polyamin-Polymer, umgesetzt mit einer epoxidierten Halohydrin-Verbindung unter Bildung von tertiären und quaternären Amingruppen auf der Dimer-Oberfläche.

2. Zusammensetzung nach Anspruch 1, bei welcher das Dimer ausgewählt wird aus der Gruppe, bestehend aus Octyl-, Decyl, Dodecyl-, Tetradecyl-, Hexadecyl-, Octadecyl-, Eicosyl-, Docosyl-, Tetracosyl-, Phenyl, Benzyl-beta-naphthyl und Cyclohexyl-Dimere; aus Montansäuren, Napthensäure, delta-9,10-Decylensäure, delta-9,10-Dodecylensäure, Palmitoleinsäure, Oleinsäure, Ricinolsäure, Linoleat, Linolsäure und Oleostearinsäure, hergestellte Dimere; und hergestellte Dimere aus natürlichen Fettsäuregemischen, wie sie aus Kokosnußöl, Babassuöl, Palmkernöl, Palmöl. Olivenöl, Erdnußöl, Rapsöl, Rinderfett und Schweinefett erhalten werden, sowie Mischungen der vorgenannten.

3. Zusammensetzung nach Anspruch 1, bei welcher das epoxidierte Halohydrin Epichlohydrin ist.

4. Verfahren zur Herstellung eines mit einem kationischen Polymer oberflächenbehandelten Füllstoffes zur Papierherstellung, welches verfahren umfaßt: Zusetzen von etwa 0,1 bis etwa 10,0 Gewichtsprozent eines kationischen Polymers, welches ein Dimer der allgemeinen Formel ist: worin R eine Kohlenwasserstoffgrupppe ist, ausgewählt aus der Gruppe, bestehend aus Alkyl mit mindestens 8 Kohlenstoffatomen, Cycloalkyl mit mindestens 6 Kohlenstoffatomen, Aryl, Aralkyl und Alkaryl, und das Dimer kationisch gemacht wurde durch Behandlung mit mindestens einem Polyamin-Amid und einem Polyamin-Polymer, umgesetzt mit einer epoxidierten Halohydrin-Verbindung unter Bildung von tertiären und quaternären Amingruppen auf der Dimer-Oberfläche; zu einer etwa 1 % bis etwa 76 % Feststoffe enthaltenden Füllstoff-Aufschlämmung, indem die Aufschlämmung unter Rühren bei einer Temperatur von etwa 5 °C bis etwa 70 °C und bei einem pH-Wert von weniger als etwa 10 gehalten wird, um das Füllstoffverhalten zu verbessern.

5. Verfahren nach Anspruch 4, bei welchem die Menge des zur Aufschlämmung zugesetzten Polymers in direkter Beziehung zur Oberfläche des Füllstoffes steht.

6. Verfahren zum Verbessern der Papierherstellung, indem mindestens eines der Ergebnisse zum Reduzieren der erforderlichen Leimungsmenge erzielt wird, Aufrechthalten des Leimungsgehaltes über die Zeit, Verbessern der Handhabungseigenschaften einer erzeugten Papierbahn, einschließlich Wasserabgabe, Verbessern der physikalischen Eigenschaften des resultierenden Papiers, einschließend Füllstoffretention, Füllstoffverteilung, Zugfestigkeit und Oberflächenreibungskoeffizient, sowie Verbessern der optischen Eigenschaften des resultierenden Papiers, einschließend Weißgrad, Opazität und Pigment-Streukoeffizient, welches Verfahren umfaßt: Zusetzen zu einem Eintrag für die Papierherstellung von etwa 5 % bis etwa 50 Gewichtsprozent Füllstoff, der oberflächenbehandelt wurde mit etwa 0,1 bis etwa 10,0 Gewichtsprozent eines kationischen Polymers, bezogen auf die Trockenmasse des Füllstoffes, wobei das kationische Polymer ein Dimer der allgemeinen Formel ist: worin R eine Kohlenwasserstoffgrupppe ist, ausgewählt aus der Gruppe, bestehend aus Alkyl mit mindestens 8 Kohlenstoffatomen, Cycloalkyl mit mindestens 6 Kohlenstoffatomen, Aryl, Aralkyl und Alkaryl, das kationisch gemacht wurde durch Behandlung mit mindestens einem Polyamin-Amid und einem Polyamin-Polymer, umgesetzt mit einer epoxidierten Halohydrin-Verbindung unter Bildung von tertiären und quaternären Amingruppen auf der Dimer-Oberfläche.

## Revendications

1. Composition qui comprend une charge de fabrication du papier choisie dans le groupe constitué du carbonate de calcium naturel finement broyé provenant d'une roche calcaire, du carbonate de calcium précipité, de l'argile, du dioxyde de titane, du talc, de pigments de silice/silicate et des associations de ces derniers, laquelle charge a été traitée à la surface par environ 0,1 à environ 10,0 % en masse d'un polymère cationique par rapport à la masse sèche de la charge, dans laquelle le polymère cationique est un dimère de formule générale : dans laquelle R est un groupement hydrocarboné choisi dans le groupe constitué d'un alkyle ayant au moins 8 atomes de carbone, d'un cycloalkyle ayant au moins 6 atomes de carbone, d'un aryle, d'un aralkyle et d'un alcaryle, le dimère ayant été rendu cationique par un traitement avec au moins un élément parmi un polyaminoamide et un polymère polyamine réagi avec un composé halohydrine époxydée pour former des groupements amines tertiaires et quaternaires sur la surface du dimère.

2. Composition selon la revendication 1, dans laquelle on choisit le dimère dans le groupe constitué d'un dimère octylique, décylique, dodécylique, tétradécylique, hexadécylique, octadécylique, eicosylique, docosylique, tétracosylique, phénylique, benzyl-β-naphtylique et cyclohexylique, de dimères produits à partir d'acides d'exploitation, de l'acide naphténique, de l'acide δ-9,10-décylénique, de l'acide δ-9,10-dodécylénique, de l'acide palmitolique, de l'acide oléique, de l'acide ricinoléique, du linoléate, de l'acide linoléique et de l'acide oléostéarique, ainsi que des dimères produits à partir de mélanges d'acides gras naturels tels que ceux obtenus à partir de l'huile de noix de coco, de l'huile d'attalée, de l'huile de semence de palmier, de l'huile de palme, de l'huile d'olive, de l'huile d'arachide, de l'huile de colza, du suif de boeuf et du lard, ainsi que des mélanges de ces derniers.

3. Composition selon la revendication 1, dans laquelle l'halohydrine époxydée est l'époxychlorhydrine.

4. Procédé de préparation d'une charge de fabrication du papier traitée à la surface par un polymère cationique, lequel procédé comprend l'ajout d'environ 0,1 à environ 10,0 % en masse d'un polymère cationique qui est un dimère de formule générale : dans laquelle R est un groupement hydrocarboné choisi dans le groupe constitué d'un alkyle ayant au moins 8 atomes de carbone, d'un cycloalkyle ayant au moins 6 atomes de carbone, d'un aryle, d'un aralkyle et d'un alcaryle, lequel a été rendu cationique par un traitement avec au moins un élément parmi un polyaminoamide et un polymère polyamine réagi avec un composé halohydrine époxydée pour former des groupements amines tertiaires et quaternaires sur la surface du dimère, à une suspension épaisse de charge contenant entre environ 1 % et environ 76 % de solides tout en maintenant la suspension épaisse sous agitation à une température comprise entre environ 5°C et environ 70°C, ainsi qu'à un pH inférieur à environ 10 de manière à améliorer la performance de la charge.

5. Procédé selon la revendication 4, dans lequel la quantité du polymère ajouté à la suspension épaisse est directement corrélée à la surface de la charge.

6. Procédé d'amélioration de la fabrication du papier en réalisant au moins l'un des résultats consistant à réduire la quantité du collage nécessaire, à maintenir la teneur du collage en fonction du temps, à améliorer les propriétés de manipulation d'une nappe de papier formée, à inclure la libération de l'eau, à améliorer les propriétés physiques du papier résultant, à inclure la rétention de la charge, la distribution de la charge, la résistance à la traction et le coefficient de friction à la surface, ainsi qu'à améliorer les propriétés optiques du papier résultant comprenant l'éclat, l'opacité et le coefficient de dispersion du pigment, lequel procédé comprend l'ajout d'environ 5 à environ 50 % en masse d'une charge qui a été traitée à la surface par environ 0,1 à environ 10,0 % en masse, par rapport à la masse sèche de la charge, d'un polymère cationique qui est un dimère de formule générale : dans laquelle R est un groupement hydrocarboné choisi dans le groupe constitué d'un alkyle ayant au moins 8 atomes de carbone, d'un cycloalkyle ayant au moins 6 atomes de carbone, d'un aryle, d'un aralkyle et d'un alcaryle, lequel a été rendu cationique par un traitement avec au moins un élément parmi un polyaminoamide et un polymère polyamine réagi avec un composé halohydrine époxydée pour former des groupements amines tertiaires et quaternaires sur la surface du dimère pour un chargement de fabrication du papier.
